

## UNITED STATES PATENT OFFICE

1,987,295

## COMMERCIAL BLASTING EXPLOSIVE

Roy Linden Hill, Wilmington, Del., assignor to  
Atlas Powder Company, Wilmington, Del., a  
corporation of Delaware

No Drawing. Application May 18, 1933,  
Serial No. 671,777

3 Claims. (Cl. 52—10)

My invention is concerned solely with commercial blasting explosives of the propulsive, rather than detonating, type which contain sodium nitrate, carbon and sulphur, i. e. with explosives, as described, which may function by mere ignition, as with a flame, and do not require the application of impact or shock to cause their proper functioning. It is further concerned solely with such explosives in hardened masses 10 in cartridge form in which the intended individual hardened portions are at least one inch long and seven-eighths inch in diameter. Practically, it is concerned with the current, so-called pellet powder of commerce and the molded product as described in the patent application of 15 James E. Slusser, Serial No. 532,341. The word "intended" above is used advisedly, because cartridges may contain smaller particles resultant from accidental breakage or erosion and yet be 20 within the scope of my invention.

An important object of my invention is an increase in strength of explosives as described without material increase in burning speed. In fact, in usual application of the invention the theoretical situation indicates no increase or even a decrease in burning speed. Incidental objects 25 are the accomplishment of the increased strength in an economical manner, without increased hazard, and by means of a material that is in 30 plentiful and continued supply.

The Slusser application above referred to discloses a molded black powder, wherein the body of powder is in such form and size as to bring about very advantageous results.

So-called pellet blasting powder is a comparatively new development insofar as the United States is concerned and the Slusser molded powder is a very recent development insofar as the entire world is concerned. Both types have involved many new factors of manufacture, properties, application and economy as compared with the old, conventional grain blasting powder. Very important among the new factors are those controlling blasting strength conditions both in themselves and together with the requirements of producing lump coal and coal with reduced 45 "checking" and shattering.

Broadly stated my invention resides in combining the essential ingredients of a desirable 50 form of black blasting powder with colloided nitrocellulose and in the form of a molded homogeneous mass of such size as to yield the highly important technical results hereinafter set forth.

I am aware of proposals for increasing the 55 strength of grain powder of the general nature

of black blasting powder, and of military explosives of a somewhat analogous composition. For example, the prior art has proposed the admixture of finished grains of colloided nitrocellulose with finished grains of black blasting powder. Such a procedure would be obviously usually unsatisfactory and uneconomical for my purpose for various reasons, among which are that my powder may never exist in grain form and desirably should avoid the extra operations of drying and blending finished individual grains before proceeding to the operations of forming my hardened masses of above prescribed sizes. Further the prior art suggests mixtures of uncolloided, merely nitrated cellulose with military black powder. To follow this procedure would be entirely uneconomical for my purpose because merely nitrated cellulose is always a primary and never a waste or salvage product and especially because it would defeat my primary object of 10 strength increase without speed increase. Uncolloided nitrocellulose will increase the speed of black powder up to, under certain conditions of amount and type of admixture, even a detonating effect. Also, uncolloided nitrocellulose could not 15 be introduced economically to my powders without greatly increased hazard. Further, it has been proposed to increase the strength of black powder by the introduction of ammonium nitrate. The proposed perchlorates increase 20 hygroscopicity, burning speed, hazard and cost.

Accordingly, my investigations and experiments convinced me that in no prior art were there satisfactory means for increasing the strength of my new types of commercial blasting 25 powder consistent with economy, safety, manufacturing convenience and accomplishment of desired powder quality and blasting effects.

It is well known that there are, annually, relatively large quantities of smokeless powder—40 colloided nitrocellulose—rejected as unfit for further military use. Some forms are colloided by means of non-explosive solvents as ether-alcohol; others by means of explosive solvents as nitroglycerine. These rejected powders may, at 45 times, be obtained at very low cost.

Specifically, my invention consists in the application of colloided nitrocellulose, as distinguished from merely nitrated cellulose or nitrocellulose applied in liquid solution in a 50 solvent, to commercial blasting powder of structure, composition and particle size previously described, in a manner to produce an important strength increase economically, conveniently and without increased burning speed and hazard. It 55

also includes the product resulting from the foregoing practice. My preferred method of manufacture involves no addition to standard equipment at mills manufacturing the types of 5 powder concerned.

That there may be no question regarding the theory of my invention I will explain as follows before discussing the detailed application of the same. It is well known that colloided nitrocel- 10 lulose functions in an entirely different manner from merely nitrated cellulose and obviously is the only form of nitrocellulose that is practical for the practice of my invention which is the development of new forms of blasting powder of 15 greatly increased strength without increase in burning speed; in other words, the desirable form of strength increase resultant from increased gas volume, rather than the usually undesirable form of seaming, but not actual, 20 strength increase resultant from speed of burning increases which do not effect an actual increase of total strength, but merely a more rapid gas evolution with the consequently greater dis- 25 integrating action, which is undesirable for most applications of blasting powder. It is obviously 30 within the scope of my invention to blend the colloided nitrocellulose by any preferred mechanical method to any preferred final product with the normal blasting powder ingredients 35 within the limits previously cited, since there is, in no case, a chemical reaction during fabrication, but a mere mechanical mixture, whatever the original and final status of the individual ingredient particles and whatever the mixing and drying methods.

In practice, I may proceed as follows: Assume 40 wheel mill incorporators of a capacity of 500 lbs. of powder and a wish to use 10% of my strengthening addition. I place 50 lbs. of wet colloided nitrocellulose in any form in the incorporator and run the wheels on it until it is of the desired 45 particle size for the particular purpose then involved. I may immediately add the composition containing sodium nitrate, carbon and sul- 50 phur of any preferred moisture content and continue the wheeling operation. Water may be allowed to decrease by evaporation or increase, by addition, at will. The time of wheeling is incidental, dependent upon the grade of final prod- 55 uct immediately sought. The product from the incorporation may be packed into molds, re- 60 moved therefrom, dried and wrapped or inserted into the ultimate cartridge containers or it may be immediately packed in the ultimate 65 containers and dried therein. These ultimate containers may be simple paper wrappers or tubes as disclosed in the Slusser application. Where 70 a low density, highly aerated product is desired, which indicates that packing intensity would be low and the molded product of insufficient mechanical stability to stand removal from molds and drying without breaking up, I prefer the second procedure. In the former case, intensity of pressing in the molds is the principal factor 75 in a hard, permanently formed final product. In the latter case, crystallization of the water soluble content of the powder is the important factor in reaching an equivalent result, indicating that a higher moisture content in the powder is preferable in the latter case.

It will be obvious that, in either case, the incorporator product may be subjected to any desired change in physical condition, such as grain- 80 ing, prior to molding. It will also be obvious 85 that my colloided nitrocellulose may be partially

or wholly preprepared as to structure before going under the wheels or may be mixed with the other ingredients prior to, during or after wheeling. It is equally obvious that the nature of the incorporator may be varied and other conditions 5 may be varied to suit. The amount of colloided nitrocellulose used is dependent entirely upon the desired strength of the ultimate product. Generally, an addition of 10% colloided nitrocellulose 10 will increase the strength of the ultimate product by about one-third as compared with the same product without the colloided nitrocellulose.

In the field of the old, conventional grain blasting powder it was possible to vary the blasting 15 action by variation in grain size through a wide range. This was not resultant from an increase in total strength, but a mere change in time of gas evolution from the powder. The new forms of molded blasting powder present 20 no such capacity for adjustment to particular 25 conditions. Consequently, it has not been possible to vary the blasting actions of these new forms to suit the coal, for instance, that is to be blasted. The result has been a limited adaptability, some blasting being served perfectly and other blasting poorly. Truly, there is a difference 30 between the pellet powder and the so-called Slusser powder, both previously described, the difference resulting from widely different manufacturing methods, but this only presents two 35 types whereas there are innumerable variations in coal seams, coal structures and types of blasted coal desired. It is true that manufacturers of pellet powder have issued up to three or four different grades, but this has been more an expedient than a procedure of practical consequence because the grades by test are very frequently found to overlap one another, or to approach one another so closely that there is no practical difference. Expedients used in efforts 40 to vary the characteristics of pellet powders have been varied wheeling or incorporating times, varied physical conditions of the individual ingredients prior to wheeling, various particle sizes and moisture contents prior to molding, varied 45 molding pressures and varied degrees of aeration; in every case ultimate results being uncertain to a high degree and the procedures costly and troublesome.

My invention permits of one systematic operating procedure, the only required variable being the amount of colloided nitrocellulose added and the desired result is definitely predictable and assured, just as in the field of high explosives the result may be assured by the nitroglycerin content added.

While theories, practices, preferred forms and limiting specifications have been given by way of examples, explanations and clarifying statements, it will be apparent that variations within 60 the scope of the disclosures and attached claims are part of my invention. From about two per cent to about 20 per cent colloided nitrocellulose is the practical range.

Colloided nitrocellulose in grain or particle 65 form is an obvious material to those skilled in the art, but definition by examples is given so that clarification may be complete. The product is instanced by smokeless powder or picture film. As a matter of economy, salvaged scrap or "break- 70 down" material is usually used in my process.

Having described my invention, what I claim is:

1. A commercial blasting unit in mass form composed of a mixture of black powder constit- 75

uents and colloided nitrocellulose material wherein the black powder constituents materially preponderate in quantity and wherein the particles of the respective ingredients are blended with each other in such manner as to form a uniform, homogeneous mixture in which the particles of the several ingredients are in close and substantially uniform contact throughout the mass, with the black powder constituents embracing and enclosing the particles of colloided nitrocellulose.

2. A commercial blasting unit in mass form of not less than one inch in length and  $\frac{1}{8}$  inch in diameter, composed of a mixture of black powder constituents and colloided nitrocellulose wherein the black powder constituents materially preponderate in quantity and wherein the particles of the respective ingredients are blended

with each other in such manner as to form a uniform, homogeneous mixture in which the particles of the several ingredients are in close and substantially uniform contact throughout the mass, with the black powder constituents embracing and enclosing the particles of colloided nitrocellulose.

3. The herein described process of preparing commercial blasting powder in mass form, which consists of molding together under at least some pressure a wet mass of black powder constituents and colloided nitrocellulose with the black powder constituents in materially preponderating quantity whereby the latter constituents are caused to embrace the colloided nitrocellulose particles.

ROY LINDEN HILL.